

## UNITED STATES PATENT OFFICE

2,104,996

## MANUFACTURE OF CORRUGATED PAPER

Charles Quincy Ives, Reading, Mass., assignor to  
Sherman Paper Products Corporation, Newton,  
Mass., a corporation of Massachusetts

No Drawing. Application March 11, 1937,  
Serial No. 130,363

11 Claims. (Cl. 92—70)

This invention relates to the manufacture of corrugated paper products such as are useful for making cartons or boxes, for wrapping fragile and other ware, for lining boxes and freight cars, etc., for which purposes they may be used as such or faced on either or both sides with flat or plane paper adhesively secured thereto. In making a corrugated paper product, it has heretofore been the practice to start with a comparatively stiff and ratty paper sheet so as to realize a finished corrugated paper product whose corrugations were of sufficient stiffness to resist breakdown or flattening out during handling, storage, and use.

15 In accordance with the present invention, there is provided a corrugated paper sheet or product whose corrugations are of marked stiffness and resistance to distorting or flattening-out influences and which, after being stretched by hand 20 or subjected to flattening pressure by the fingers, tends to recover practically completely its original corrugated form. Unlike the corrugated paper products heretofore produced, the corrugated paper sheet hereof is produced from an initially flat paper sheet wherein no attempt has necessarily been made to realize high degree of stiffness or rattle, as by the introduction of sizing or stiffening agents thereto. The starting paper sheet for the corrugated paper product hereof is 25 characterized by a substantial content of leather fiber which, although essentially a "dead" ingredient in the initially flat paper sheet in the sense that it does not contribute significantly to the stiffness or rattle of such flat sheet, is more 30 or less incipiently fused by heat during the sheet-corrugating operation so as to exert a very marked stiffening effect in the finished or corrugated paper product and at the same time to impart a high degree of resiliency to the corrugations so that they recover or spring back substantially to their original form when distorting or flattening stresses applied thereto are removed. It might be noted that in forming the 35 corrugated paper product hereof, it is necessary simply to pass the flat starting sheet between one or more pairs of corrugating rolls heated to sufficiently elevated temperature to cause the desired incipient fusion of the leather fiber content of the sheet; and upon the mere cooling of the hot corrugated sheet emerging from the nip of the corrugating rolls and the setting of its content of leather fiber from incipiently fused condition, the 40 advantageous corrugated paper product hereof results. An important advantage of the initially flat sheet used herein is that it is readily con-

formable with the need of little, if any, moisture therein as it passes into the nip of the corrugating rolls, wherefore, the corrugated sheet hereof requires little, if any, drying after the corrugating operation. It is generally preferable to pass the flat starting sheet through corrugating rolls heated to a temperature of about 300° to 400° F. in producing the corrugated paper product hereof, as the desired incipient fusion of the leather fiber content of the sheet can be effected very quickly at such temperature while substantially avoiding scorching or other injury to the cellulosic fibers.

The corrugated paper product hereof may be fabricated from starting paper sheets of various compositions, but, in any event, it is desirable that the starting or initially flat sheet have a leather fiber content of about 10 to 50%, based on its total weight, so as to provide sufficient incipiently fusible fibrous ingredient to impart the valuable qualities of stiffness and resiliency to the finished corrugated paper product hereof. Generally speaking, the starting paper sheet for the purpose hereof is preferably of a thickness of about 0.006 to 0.012", as such a sheet may be converted by the invention hereof into a finished corrugated paper product of the requisite body and mechanical properties, including tensile strength, tear resistance, etc. Because of the binding and stiffening effect of the incipiently fused leather fiber content in the finished corrugated paper product, it is unnecessary to use high grade cellulosic fibrous material along with the leather fiber in the beater or papermaking furnish to realize at a sheet thickness of about 0.006 to 0.012" in the finished corrugated paper product the requisite mechanical properties. The fact is that even the cheapest or waste cellulosic materials, including such waste papers as glassine, parchment, wax papers, and others of relatively low fiber strength when disintegrated or reduced to pulp, may be used along with the appropriate proportion of leather fiber in producing by the invention hereof an eminently satisfactory corrugated paper product having a thickness no greater than about 0.06 to 0.012".

The invention hereof will now be described in terms of a specific example of procedure involving the use of a beater furnish composed essentially of mixed waste papers and scrap leather or leather-board. To the usual beater or Hollander engine was added 1500 parts by weight of various waste papers, namely, about 1000 parts of mixed waste papers sometimes termed "floor sweepings" and about 500 parts of waste kraft and manila papers; 50

and about 275 parts of previously shredded or dis-integrated tanned scrap sole leather was also added to the beater along with sufficient water to ensure free circulation of the beater charge or 5 contents. The beater charge was beaten or dis-integrated for a period of about an hour or more, with gradual lowering of the beater roll at the end of the beating operation so as to ensure a smooth finished stock or papermaking furnish 10 which could be formed into a sheet of the desired uniform texture on a Fourdrinier or equivalent papermaking machine. In the course of the beating operation, for instance, at the end stages thereof, it is preferable to add about 20 to 30 15 pounds of lime to the beater charge for the purpose of facilitating the disintegration or defiberization of such residual clumps or pieces of paper, such as waxed paper, that may resist complete defiberization. The lime apparently promotes a 20 dispersion of the wax content of the residual waxed paper pieces and simultaneously to cause individualization or separation of the fibers constituting such pieces. Again, the lime, evidently by reason of reaction with the leather fibers 25 and/or their content of tanning agent, generates a substantially uniform brown coloration throughout the beaten stock, which coloration is desirable in that the paper sheet made from the stock has a brown or tannish hue reminiscent of kraft 30 paper and thus attractive to the consumer. Such brown coloration of the stock ensues, irrespective of such varied color waste papers as may constitute the raw material of the beater furnish; and such coloration is sufficiently potent or dominating 35 to offset or mask the varied colors of the waste papers, which varied colors, if permitted to persist in the finished paper product, would make for a heterogeneously or irregularly colored paper of poor or unattractive appearance.

40 The lime-treated beaten stock is preferably jordaned prior to its delivery to the stock chest of the papermaking machine wherein the stock may be diluted with water from a beater or Jordan consistency of, say, about 5% to a papermaking 45 consistency of about  $\frac{1}{2}\%$ . The stock is formed on the papermaking machine into a sheet of a thickness of preferably about 0.009" and wound up as delivered from the dry end of the papermaking machine into parent rolls for transfer to 50 the corrugating machine.

55 The paper sheet may be progressively unwound from a parent roll and run through a corrugating machine whose corrugating rolls are internally heated by steam or other suitable heating medium to a temperature of, say, about 340° to 350° F. As already indicated, it is unnecessary to moisten 60 the paper sheet preparatory to its being progressively run through the corrugating rolls maintained at such temperature, since the sheet very nicely assumes the fluted peripheral configuration of the corrugating rolls without any tendency whatever to be embrittled, crushed, or torn in the flutes or teeth of the rolls. The corrugated sheet 65 progressively issuing from the nip of the corrugating rolls is preferably placed under little tension or restraint immediately after its issuance from the corrugating nip, but, as it gradually cools down to room temperature and its incipiently fused leather fiber component and its corrugations 70 stiffen or set, the slack in the sheet may be taken up and the sheet may be accumulated under tension in roll form or, prior to such accumulation, be faced under tension on either or both sides 75 with a plane paper sheet, which may be adhe-

sively secured to the crests of the corrugations, as ordinarily.

It is to be understood that the principles of the present invention extend to the use of paper sheets made from furnishes containing cellulosic fibers of all sorts and treated or processed otherwise than in the specific example hereinbefore given. Thus, the cellulosic fiber component of the beater furnish may be any one or a mixture of a wide variety of virgin fibers, such as kraft, 10 sulphite, or other chemical wood pulp, mechanical wood pulp, newsprint, rags, etc.; and the leather fiber component of the furnish may be had from scrap leatherboard, waste leather, or the like, which may be reduced or disintegrated 15 to pulp form in the presence of water in the beater engine prior to the admixture therewith of the cellulosic fiber component. In some instances, it may be desirable to replace some or most of the cellulosic fiber component of the papermaking 20 furnish with such specific fibers as asbestos and/or wool in order to impart special or specifically desired properties in the finished corrugated sheet hereof. It is preferable to use lime as the promoter of disintegration of refractory papers such 25 as waste waxed paper and as the chemical for generating the tan color throughout the stock by reaction with the defiberized tanned leather scrap and/or its content of tanning agent. In this latter connection, it might be noted that while such 30 stronger alkalies as caustic soda might be used in lieu of lime for such latter purpose, they are more expensive than lime and tend to gelatinize or dissolve the leather fibers and thus to lead to a 35 paper sheet of unduly high initial stiffness or brittleness coupled with unduly low tear resistance such as give rise to the danger of breakage or 40 rupture of the sheet during the corrugating operation.

I claim:

1. A corrugated paper sheet containing, besides cellulose fiber, leather fiber set from incipiently fused condition and contributing marked stiffness and resiliency to the corrugations of said sheet.

2. A corrugated paper sheet of a thickness of 0.006 to 0.012 inch and containing, besides cellulose fiber, leather fiber set from incipiently fused condition and contributing marked stiffness and resiliency to the corrugations of said sheet.

3. A corrugated paper sheet containing leather fiber in the amount of about 10% to 50%, based on the weight of the sheet, set from incipiently fused condition and contributing marked stiffness and resiliency to the corrugations of said sheet.

4. A corrugated paper sheet of a thickness of about 0.006 to 0.012 inch and containing leather fiber in the amount of about 10% to 50%, based on the weight of the sheet, set from incipiently fused condition and contributing marked stiffness and resiliency to the corrugations of said sheet.

5. A method which comprises forming a paper sheet from a papermaking furnish containing, besides cellulose fiber, leather fiber in substantial amount; and corrugating the resulting paper sheet under sufficient heat to cause incipient fusion of said leather fiber.

6. A method which comprises forming a paper sheet from a papermaking furnish containing, besides cellulose fiber, leather fiber in substantial amount; and corrugating the resulting paper sheet at a temperature of about 300° to 400° F.

7. A method which comprises forming a paper sheet from a papermaking furnish containing

about 10% to 50% leather fiber, based on the weight of the solid ingredients of said furnish; and corrugating the resulting paper sheet at a temperature of about 300° to 400° F.

5 8. A method which comprises forming a paper sheet of a thickness of about 0.006 to 0.012 inch from a papermaking furnish containing about 10% to 50% leather fiber; and corrugating the resulting paper sheet in substantially dry condition at a temperature of about 300° to 400° F.

10 9. A method which comprises incorporating alkali into a paper making furnish containing a substantial amount of leather fiber in admixture with cellulosic fiber, forming a paper sheet from said alkali-treated furnish, and corrugating the resulting paper sheet under sufficient heat to cause incipient fusion of said leather fiber.

15 10. A method which comprises incorporating

lime into a papermaking furnish containing tanned leather fiber in the amount of about 10% to 50% by weight of the solid ingredients of said furnish, forming a paper sheet from said lime-treated furnish, and corrugating the resulting 5 paper sheet under sufficient heat to cause incipient fusion of said leather fiber.

11. A method which comprises incorporating lime into a papermaking furnish containing essentially beaten waste paper and defiberized 10 scrap sole leather, said leather fiber constituting about 10% to 50% by weight of the solid ingredients of said furnish, forming said lime-treated furnish into a paper sheet of a thickness of about 0.006 to 0.012 inch, and corrugating the resulting 15 paper sheet in substantially dry condition at a temperature of about 300° to 400° F.

CHARLES QUINCY IVES.